



US006341836B1

(12) **United States Patent**  
Koike et al.

(10) **Patent No.:** US 6,341,836 B1  
(45) **Date of Patent:** Jan. 29, 2002

(54) **WATER-REPELLENT COATING AND METHOD FOR FORMING SAME ON THE SURFACE OF LIQUID JET**

(75) Inventors: **Shuji Koike, Kawasaki; Masayuki Sasaki, Inagi; Tomoyuki Akahoshi, Kawasaki, all of (JP)**

(73) Assignee: **Fujitsu Limited, Kawasaki (JP)**

(\*) Notice: Subject to any disclaimer, the term of this patent is extended or adjusted under 35 U.S.C. 154(b) by 0 days.

(21) Appl. No.: **09/484,036**

(22) Filed: **Jan. 18, 2000**

(30) **Foreign Application Priority Data**

Mar. 17, 1999 (JP) ..... 11-071202

(51) **Int. Cl.<sup>7</sup>** ..... **B41J 2/135**

(52) **U.S. Cl.** ..... **347/20**

(58) **Field of Search** ..... 347/20, 44, 45, 347/46, 47; 428/446

(56) **References Cited**

U.S. PATENT DOCUMENTS

5,502,470 A \* 3/1996 Miyashita et al. ..... 347/45  
5,863,371 A 1/1999 Takemoto et al.  
5,919,572 A \* 7/1999 Blum et al. ..... 428/446

FOREIGN PATENT DOCUMENTS

|    |              |         |
|----|--------------|---------|
| EP | 0 506 128 A1 | 9/1992  |
| JP | 56-166085 A  | 12/1981 |
| JP | 59-47399 A   | 3/1984  |
| JP | 59-106918 A  | 6/1984  |

|    |            |         |
|----|------------|---------|
| JP | 59-176054  | 10/1984 |
| JP | 4-339662 A | 11/1992 |
| JP | 5-4344 A   | 1/1993  |
| JP | 5-193140 A | 8/1993  |
| JP | 6-246921 A | 6/1994  |
| JP | 6-344560   | 12/1994 |
| JP | 7-171964 A | 7/1995  |
| JP | 8-142334 A | 6/1996  |
| JP | 8-244233   | 9/1996  |
| JP | 9-076492 A | 3/1997  |
| JP | 09104109   | 4/1997  |
| JP | 9-31880 A  | 5/1997  |

OTHER PUBLICATIONS

Patent Abstracts of Japan, vol. 1999, No. 03 (Mar. 31, 1999) & JP 10 323984 A (Dec. 8, 1998) translation \*abstract\*.

Patent Abstracts of Japan, vol. 1995, No. 03 (Apr. 28, 1995) & JP 06 344560 A (Dec. 20, 1994) \*abstract\*.

Patent Abstracts of Japan, vol. 014, No. 052 (Jan. 30, 1990) & JP 01 280566 A (Nov. 10, 1989) \*abstract\*.

Patent Abstracts of Japan, vol. 012, No. 197 (Jun. 8, 1988) & JP 63 003963 A (Jan. 8, 1988) \*abstract\*.

\* cited by examiner

Primary Examiner—Ana T. N. Vo

(74) Attorney, Agent, or Firm—Armstrong, Westerman, Hattori, McLeland & Naughton, LLP

(57) **ABSTRACT**

A water-repellent coating having a higher wiping resistance against a wiper and capable of being formed by a more simplified process than was previously possible. The method of forming the water-repellent coating comprises a flat hard body and a plating-processed fluoric polymer which are formed on a nozzle plate having a nozzle as a substrate around the nozzle.

**10 Claims, 7 Drawing Sheets**





FIG. 1



FIG. 2



FIG. 3



FIG. 4



FIG. 5

(A)



(E)



(B)



(C)



(D)



FIG. 6



FIG. 7





FIG. 10

**WATER-REPELLENT COATING AND  
METHOD FOR FORMING SAME ON THE  
SURFACE OF LIQUID JET**

**BACKGROUND OF THE INVENTION**

The present invention relates to compositions of water-repellent coatings on the surface of liquid jet nozzles and in particular a nozzle plate for an inkjet printer.

Among inkjet heads, those using a piezo-electric element have recently become more and more popular for their high energy-efficiency, etc. This kind of inkjet head typically comprises a piezo-electric element, one common ink chamber with ink supplied from outside and stored therein, a plurality of pressure chambers connected to the piezo-electric element and a nozzle plate connected to the pressure chambers so that a nozzle is connected to each pressure chamber. Each pressure chamber that is connected each corresponding ink feed path to the common ink chamber receives ink from the common ink chamber, increases an internal pressure by utilizing a deformation of the piezo-electric element, and thereby jets ink from the nozzle.

On the surface of the nozzle plate (opposite to the pressure chamber) a water-repellent coating is typically formed around the nozzle. The water-repellent coating has the following exemplary effects. First, the water-repellent coating serves to stabilize a flying direction of ink jettet from the nozzle. Without the water-repellent coating, onto the nozzle plate surface is adhered the ink spouted from the pressure chamber, the ink adhered onto the nozzle plate like this pulls the next ink jettet continuously, and thereby bends the flying direction of ink and prevents from flying straight in a desired direction. Secondly, the water-repellent coating serves to smooth a wiping process. After a printing operation is completed, the inkjet head usually undergoes a backup process that eliminates dirt from the nozzle. In the backup process, a suction pump contacts the nozzle and sucks out dirt therein, and at the same time the ink in the nozzle adheres onto the surface of the nozzle plate. Thus, the wiping process that a wiper such as rubber blade, etc. wipes ink on the nozzle surface follows. In that event, without the water-repellent coating, the ink adhered onto the nozzle plate surface after the backup process could not successfully be wiped out and would remain on the nozzle plate surface. Consequently, the subsequently flying direction of ink is bent and printing quality is adulterated with impure or diluted color if the remaining ink is different in color from the subsequently flying ink.

For the forgoing effects, it is inevitable for inkjet head to form the water-repellent coating. In addition, a conventional water-repellent coating has a fluoric polymer of high water repellency as a main ingredient.

However, the fluoric polymer is soft and less adhesive to a substrate, and thus is likely to flaw, abrasion or scratch (i.e. low wiping-resistant); therefore, its anticipated water repellency can not be continuously maintained. Accordingly, it has been desired to form a water-repellent coating that has a fluoric polymer as a main ingredient and is continuously usable about one hundred thousand times.

Conventionally, it has been suggested for example that a fluoric polymer is plated and a subsequent heating process melts the fluoric polymer adhered onto the plated surface, forms a coating and thereby improves its wiping resistance. This process, however, involves a problem that the coating, even if it is formed, is worn out shortly by a plural of frictions and its water repellency lowers. On the other hand, it has also been suggested to form a member around the

liquid jet in concave shape and avoid the fluoric coating around the nozzle from scratched by a friction. The unlevelling process, however, increases its person-hours and costs.

**BRIEF SUMMARY OF THE INVENTION**

Accordingly, it is a general object of the present invention to provide a novel and useful water-repellent coating and method of forming the water-repellent coating in which the above disadvantages are eliminated.

More specifically, it is an exemplified object of the present invention to provide a water-repellent coating that has higher wiping resistance relative to a wiper and is formed by a more simplified process than was previously possible, and a method of forming such a water-repellent coating.

In order to achieve the above object, a print head according to claim 1 comprises a nozzle plate having a nozzle which jets ink, and a water-repellent coating that is formed on the nozzle plate as a substrate around the nozzle and comprises a hard body and a fluoric polymer formed by a plating process. According to the print head claimed in claim 1, water repellency of the fluoric polymer works against liquid like ink, etc. jettet from the nozzle, and the hard body enhances wiping resistance of the fluoric polymer.

A print head as set forth in claim 2 that depends upon claim 1 comprises a water-repellent coating including the hard body in a flat shape. Thus, according to the print head claimed in claim 2, the hard body is less likely to fall off than a spherical shaped one and serves to maintain wiping resistance for a long time.

A print head as set forth in claim 3 that depends upon claim 1 comprises a water-repellent coating including the hard body having a major axis of 1  $\mu\text{m}$  or smaller in its particle diameter. According to the print head claimed in claim 3, the hard body having a big particle diameter never prevents a nozzle plate surface from being smoothly wiped. A print head as set forth in claims 4 and 5 that depends upon claim 1 comprises a water-repellent coating having the hard body including a boron nitride boron nitride single crystal. Therefore, according to the print head claimed in claims 4 and 5, the boron nitride or boron carbide single crystal intrinsically having the advantage of a flat shape requires no additional process to deform the hard body into a flat shape.

A print head as set forth in claims 6 and 7 that depends upon claim 1 comprises a water-repellent coating employing an electrolytic or electroless plating process as the plating process. Accordingly, the print head claimed in claims 6 and 7 has the advantage of requiring no special plating process.

A recording device as set forth in claim 8 comprises a print head and a driving device which drives the print head wherein the print head includes a nozzle plate having a nozzle which jets ink and a water-repellent coating which is formed on the nozzle plate as a substrate around the nozzle and comprises a hard body and a fluoric polymer formed by a plating process. According to the recording device claimed in claim 8, water repellency of the fluoric polymer works against liquid like ink, etc. jettet from the nozzle, and the hard body enhances wiping resistance of the fluoric polymer.

A method of forming a water-repellent coating as set forth in claim 9 comprises the steps of forming on a nozzle plate a first resist which is open only around a nozzle of the nozzle plate, forming a first layer of a plated fluoric polymer by a first plating process via the first resist, forming a second resist, adding a hard body to a first layer by a second plating process, and removing the first and second resists. According to the method of forming a water-repellent coating claimed in this claim, the hard body is allowed to protrude

from the water-repellent coating surface because the water-repellent coating is formed on the nozzle plate as a substrate. A method claimed in claim 10 that depends on claim 9 further comprises the step of heating the water-repellent coating until its water repellency becomes enough to make a contact angle of ink containing 10% of alcohol 60 degrees or larger. By the heat treatment, the fluoric polymer melts and taking in the additive hard body.

Other objects and further features of the present invention will become readily apparent from the following description and accompanying drawings.

#### BRIEF DESCRIPTION OF DRAWINGS

FIG. 1 is a schematic sectional view for explaining a composition of a water-repellent coating of the present invention.

FIG. 2 is a schematic sectional view illustrating a variation of the water-repellent coating shown in FIG. 1 or a state after a predetermined period of use.

FIG. 3 is an enlarged view of a portion circled in a solid line in FIG. 2.

FIG. 4 is an aschematic sectional view for explaining a composition of a water-repellent coating having a spherical hard body relative to the water-repellent coating in FIG. 1 having a flat hard body.

FIG. 5 is a schematic sectional view for explaining a state in which the spherical hard body in FIG. 4 is fallen down.

FIG. 6A-FIG. 6E are flow sectional diagrams for explaining one example of a method of forming the water-repellent coating shown in FIG. 1.

FIG. 7A-FIG. 7E are flow sectional diagrams for explaining another example of a method of forming the water-repellent coating shown in FIG. 1.

FIG. 8 is an exploded perspective view of a completed inkjet head 300.

FIG. 9 is a partially enlarged side view of an inkjet head 300.

FIG. 10 is a perspective overview of a recording device according to the present invention.

#### DETAILED DESCRIPTION OF THE INVENTION

Referring now to FIGS. 1 to 3 inclusive, a description will be given of a water-repellent coating 100 according to the present invention. FIG. 1 is a schematic sectional view for explaining a composition of a water-repellent coating 100 of the present invention. FIG. 2 is a schematic sectional view of a water-repellent coating 100a showing an exemplified variation or a state after a predetermined period of use. FIG. 3 is an enlarged view of a portion circled in a solid line in FIG. 2. In each drawing, those elements designated by the same reference numeral denote the same elements, and a duplicate description thereof will be omitted. Those elements designated by the same reference numeral with a variety of alphabetical letters attached thereto denote the same kinds of elements but are distinguished from each other by alphabets and are comprehensively designated by simple reference numerals.

The water-repellent coatings 100 and 100a are, for example, 1 through 2  $\mu\text{m}$  thick and are formed around a nozzle 12 on the surface of a nozzle plate 10. FIG. 1 is an enlarged sectional view around a nozzle (hole) 12 applicable to a print head 300 which will be described later (e.g. piezo-type inkjet head and a bubble jet-type inkjet head).

The nozzle plate 10 comprises the nozzles 12 each having a straight portion 14 and a taper portion 16, to the number corresponding to a predetermined resolution. The nozzle 12 does not necessarily include both of the straight portion 14 and the taper portion 16 but may include only one of them. A portion defined by the straight portion 14 is an opening portion 18 of the nozzle 12 where a meniscus 20 of ink is formed. The nozzle plate 10 is connected to a pressure chamber plate 30, and the pressure chamber plate 30 is provided with an ink chamber as will be described later.

The water-repellent coatings 100 and 100a comprise a fluoroplastic coating 102, a fluoroplastic particle 104, a nickel base 106 and a flat hard body 108. The water-repellent coating 100 shown in FIG. 1 is different from the water-repellent coating 100a shown in FIG. 2 in whether the flat hard body 108 is partially protruded from the fluoroplastic coating 102.

The water-repellent coatings 100 and 100a are characteristically formed on the nozzle plate 10 as a substrate. Therefore, this invention does not adopt such a method, for example, that the water-repellent coating and the nozzle plate 10 are formed in this sequence on a plane and then the plane is removed. Because this method makes the hard body 108 unable to protrude from the fluoroplastic coating 102 as shown in FIG. 2. A projection structure of the hard body 108 as shown in FIG. 2 is suitable for preventing the fluoroplastic coating 102 from being scratched by a friction of a wiping blade (wiper) and making it possible to maintain ink water repellency for a long period.

For the fluoroplastic coating 102 and the fluoroplastic particle 104, tetrafluoroethylene resins, tetrafluoroethylene-hexafluoropropylene copolymerization resins, trifluoroethylene chloride resins, fluoro vinylidene resins, fluoro vinyl resins, PTFE, FEP, ETFE, PFA, PCTFE and PVDF are usable either singly or in the form of a mixture of two or more of them. Their average particle diameters should preferably be less than 150  $\mu\text{m}$  and in particular ranging from 0.05 to 20  $\mu\text{m}$ . In addition to the above fluoroplastic particles, as needed, other inorganic or organic precipitation polymer particulates may be formed together.

The nickel base 106 as a plating coating is added to improve adhesion. Other than nickel may be employed copper, silver, zinc, tin, cobalt and such nickel alloys as a nickel-cobalt alloy, a nickel-phosphorus alloy and a nickel-boron alloy, etc. The plating coating can be formed, for instance, by using the electrolytic plating solution or electroless plating solution in which PFA is suspended. The electrolytic plating solutions according to a variety of metal plating coatings to be deposited may be selected from an electrolytic nickel plating solution such as the Watts bath, a chloride-rich bath, a nickel sulfamate bath and a nickel borofluoride bath, etc.; an electrolytic cobalt plating solution such as a cobalt sulfate bath and a cobalt chloride bath, etc.; an electrolytic copper plating solution such as a copper sulfate bath and a copper borofluoride bath, etc.; an electrolytic lead/tin plating solution such as a lead sulfate bath, a tin sulfate bath and a lead borofluoride bath, etc. It is however preferable to employ a sulfamic acid bath having a sulfamic acid ion content of more than 0.5 mol, more desirably more than 0.8 mol especially in the light of their properties that form more precipitation and resist agitation. The electroless plating solutions may be selected from an electroless nickel plating solution, an electroless cobalt plating solution and an electroless copper plating solution, etc. using a boron compound such as a hypophosphate and a dimethyl borazon, etc. as a reducing agent.

The hard body 108 has a higher hardness than a fluoric polymer and a flat shape. The hard body 108 should pref-

erably be as water-repellent, wiping-resistant and frictionless as possible. Even though the hard body **108** has low water repellency, a heat treatment as will be described later melts the fluoric polymer, covers the hard body **108**, and thereby maintains the water repellency. The hard body **108** is added so as to promote the wiping resistance of the fluoric polymer against the wiper. Its flat shape aims at enhancing an anchor effect into the plating coating. A more specific description is now given to the enhanced anchor effect. To illustrate, suppose that a spherical hard body **208** (e.g. having more than 1  $\mu\text{m}$  in diameter) is dispersed in the water-repellent coating **200** (e.g. of about 1  $\mu\text{m}$  in thickness), as shown in FIG. 4. If the water-repellent coating **200** is wiped on its surface by a wiper **5**, the spherical hard body **208** other than having more than half of its diameter embedded in the water-repellent coating **200** is fallen down as shown in FIG. 5, so that the wiping resistance of the water-repellent coating lowers to such a level as that of the water-repellent coating having no hard body **208**. In FIG. 5, a mark left by the hard body **208** is indicated with **209**.

As the hard body **108**, are usable, for example, BN (boron nitride), boron carbide, silicon carbide, titanium carbide, tungsten carbide, graphite fluoride, alumina, glass and ceramics, etc. The boron nitride and boron carbide are suitable for the water-repellent coating of this invention in that they are dealt with in a single crystal and the single crystal is not spherical in crystal structure (the boron nitride is flat). Particularly, the boron nitride, which is used for reducing friction of a bearing, is suitable for improving sliding properties of the electroless nickel coating and increasing strength of the fluoroplastic coating **108**. When the alumina, glass, ceramics are used, they should be deformed in a flat shape. BN added for this is, for example, some 5 g/l or 10 g/l, preferably 20 g/l.

Since the additive hard body **108** is less water-repellent than the fluoric polymer, the water-repellent surface should be covered as widely with the fluoric polymer as possible. Therefore, it is necessary to increase a water-repellent portion of liquid contact surface by heating and melting the fluoric polymer after plated so as to taking in the additive.

Referring now to FIG. 6A–FIG. 6E, a description will be given of a method of manufacturing a nozzle plate with a water-repellent coating as shown in FIGS. 1 and 2. Hereupon, FIG. 6A–FIG. 6E are flow sectional diagrams for explaining one exemplified method of the water-repellent coating **100** shown in FIG. 1 or the water-repellent coating **100a** shown in FIG. 2. First, as shown in FIG. 6(A), a nozzle plate substrate **10** of a stainless steel (SUS316) plate of 100  $\mu\text{m}$  through 300  $\mu\text{m}$  thickness is processed by stamping, etching, electrical discharge machining and laser machining, etc. and is provided with a nozzle **12**. To illustrate, assume that a conic nozzle **12** is made by stamping, a straight portion **14** being 40  $\mu\text{m}$  thick and 20  $\mu\text{m}$  length, and a taper portion **16** has a taper angle of 20 degrees. A nozzle plate surface **22** is roughly ground to remove burrs left by the processing but the burrs are not completely removed.

Next, as shown in FIG. 6(B), corrosion-resistant polymer resin as a resist is filled in the processed nozzle **12**. A photosensitive liquid resist is usable as a resin member in contemplation of its subsequent removal and its machinability. This example utilizes a dry film resist (DFR) **24** of a curing acrylic resin. The DFR **24** becomes a viscous liquid by adding a sufficient heat and is easily filled in the nozzle **12**. Further, in terms of removal, water soluble DFR which may be easily removed with alkaline water solution is available.

As shown in FIG. 6(C), the nozzle plate surface **22** is drenched in a stainless etching solution and etched. On the

nozzle plate surface **22** there exist burrs left by the processing or rough grinding of the nozzle **12**, but can easily be removed by etching process. This makes it possible to omit a final finishing grinding step in processing the nozzle plate **10**, and enables a cost-reduction. In addition, a chemical grinding means, if used, may reduce a mechanical stress applied to the nozzle substrate **10** and may improve processing accuracy. The etching depth is 10  $\mu\text{m}$  and the length of straight portion **14** is 10  $\mu\text{m}$ .

Thereafter, a water washing, an electrolytic defatting, a water washing, an acid washing and a strike Ni plating are processed, and a water-repellent coating **100** is formed on the nozzle plate surface **22** with a Ni precipitation plating as shown in FIG. 6(D). The water-repellent coating **100** has the thickness not exceeding the height of the protruded DFR **24**. Then, the nozzle plate **10** is drenched in an alkaline water solution, the DFR **24** is removed as shown in FIG. 6(E), and the nozzle plate **10** with a water-repellent coating **100** becomes completed. When materials as having difficulty in being etched, such as ceramics, glass, etc. are used as the nozzle plate **10**, the grinding process (FIG. 6(C)) may be substituted by a physical means using a sandblast. In that event, a sandblast-resistant DFR **24** that includes a polyurethane resin other than an acryl resin as usual ingredients (e.g. BF series made by Tokyo Ohka Kogyo Co., Ltd.) may be employed. The physical grinding means is also applicable to a nozzle plate substrate **10** made of metal.

Like this, the water-repellent coating **100** on the nozzle plate surface **22** by Ni precipitation plating is formed along a projected portion of DFR **24**, preventing dropping into the nozzle **12**, and maintains the size accuracy of the nozzle **12** and the water-repellent coating **100**. For example, in FIG. 1, the water-repellent coating **100** is formed so that it permits dropping by making its diameter  $\phi_2$  within 3% range of the diameter  $\phi_1$  of an opening **18**. This 3% difference is for the purpose of arranging the opening of the water-repellent coating **100** and the opening **18** of the nozzle plate on almost the same side. This arrangement can prevent a deviation of ink dots, stabilize flying ink direction and provide high quality images.

Referring next to FIG. 7A–FIG. 7E, a description will be given of another method of manufacturing the nozzle plate **10** having the water-repellent coating **100**. The process shown in FIG. 7A–FIG. 7E, is a variation of the process of FIG. 6(C) and those that follow, and it is to be construed that the process indicated in FIG. 7(A) follows the process indicated in FIG. 6(B). As shown in FIG. 7(A), on the nozzle plate surface **22** is formed a liquid resist or a DFR coating **26** capable of alkaline development and removal, and then the exposure and development with a mask pattern eliminate coatings around the opening **18** on the nozzle plate surface **22**. Next, as shown in FIG. 7(B), the nozzle plate substrate **10** is drenched in an etching solution and the surface of the opening the coating **26** is ground. The etching depth can be adjusted by altering etching conditions. By adjusting the depth, the length of the straight portion **14** and the projection amount of the DFR **24** are adjusted.

As shown in FIG. 7(C), the coating **26** is removed with strong alkaline solution. In this case, the DFR **24**, which is an alkaline-resistant resist, is not eliminated and remains. After that, a water washing, an acid washing, an electrolytic defatting, a water washing and a strike Ni plating are processed. Subsequently, as shown in FIG. 7(D), Ni precipitation plating is processed on the nozzle plate surface **22** and the water-repellent coating **100** is formed. The coating thickness is so adjusted as does not exceed the projection amount of the DFR **24**. Thereafter, as shown in FIG. 7(E),

the DFR 24 are removed and eliminated with solution development-type resist removal solution.

The above manufacturing method can also provide a nozzle plate 10 having an accurate sized water-repellent coating 100, as in FIG. 6. This method, particularly as using DFR 24 as a resist member, only necessitates a heating process where an exposure process may be omitted, and is applicable at one step from the back of the nozzle plate substrate 10, whereby reducing manufacturing costs.

Description will be given of a method of manufacturing a water-repellent coating 100 shown in FIG. 1 or a water-repellent coating 100a shown in FIG. 2. First, in order to form a water-repellent plating coating only on the surface of the nozzle plate 10, other portions are masked so as not to adhere the coating. In this step, the nozzle plate 10 as a substrate is laminated at the side on which a pressure chamber 30 is formed with an alkaline development-type dry film (this exemplified embodiment utilizes  $\alpha$ -450 made by Tokyo Ohka Kogyo Co., Ltd.) on conditions of 120°C, 2.5 kgf/cm<sup>2</sup>, 0.5 m/min. This allows the dry film to break in to the taper portion 16 and the straight portion 14 of the nozzle 12. Moreover, the resist flows out of ink jet opening of the nozzle, covering a portion around the edge of the nozzle opening of a width of 1  $\mu$ m, and then the resist is hardened by a double-sided exposure.

On the other hand, in order to form a water-repellent coating with a single crystal BN (boron nitride) added thereto, prepare a fluoroplastic containing Ni plating solution (made by Hikifune Co., Ltd.) to which a BN with longitudinal particle size of 1  $\mu$ m or smaller (particles of more than 1  $\mu$ m being crushed to this size) is added at the rate of 20 g/l and coat a water-repellent plating to the nozzle plate 10 masked as described above.

The nozzle plate 10, made of stainless steel (SUS430), is drenched in 10% hydrochloric acid for three minutes, washed in water to remove an oxidized coating and is strike Ni plated to improve its plating adhesion.

The specification of the strike Ni plating is as follows.

|                                                         |                     |
|---------------------------------------------------------|---------------------|
| (1) <u>Bath composition</u>                             |                     |
| nickel chloride (NiCl <sub>2</sub> , 6H <sub>2</sub> O) | 220 g/l             |
| hydrochloric acid (HCl 35%)                             | 45 g/l              |
| (2) <u>Temperature</u>                                  | room temperature    |
| (3) <u>Electrode</u>                                    |                     |
| titanium basket (150 x 30 x 250 mm)                     |                     |
| electrolytic nickel (ø 1B x 10 mm)                      |                     |
| (4) <u>Current density</u>                              | 2 A/dm <sup>2</sup> |

After one-minute plating by using this strike Ni plating solution, the nozzle substrate is drenched in a water-washing bath and immediately commences a water-repellent plating process. The specification of the water-repellent plating is as follows.

|                                 |                     |
|---------------------------------|---------------------|
| (1) <u>Solution composition</u> |                     |
| nickel sulfamate                | 420 through 480 g/l |
| nickel chloride                 | 40 through 50 g/l   |
| boric acid                      | 30 through 40 g/l   |
| PTFE                            | 40 through 50 g/l   |
| BN                              | 20 g/l              |
| PH                              | 4.0 through 4.4     |

-continued

|                                     |                     |
|-------------------------------------|---------------------|
| (2) <u>Temperature</u>              | 42° C.              |
| (3) <u>Electrode</u>                |                     |
| titanium basket (150 x 30 x 250 mm) |                     |
| electrolytic nickel (ø 1B x 10 mm)  |                     |
| diaphragm                           |                     |
| (4) <u>Current density</u>          | 2 A/dm <sup>2</sup> |

10 The nozzle substrate is plated for three minutes by using this water-repellent plating solution. After washed in water, it is drenched in a NaOH (3 wt %) solution, removes a resist, and then after water washing and drying processes, makes PTFE into a coating adhered as a plating by a heating process at 350°C for thirty minutes. The plated coating, as shown in a photograph attached herewith, has BN particles scattered thereon, whereby preventing a convex portion of the BN particles from being scratched even though an outermost fluoroc coating is scratched by friction and abrasion of a wiper (rubber blade), so that a water-repellent effect can be maintained.

20 Referring next to FIGS. 8 and 9, a description will be given of an inkjet head 300 of the present invention. FIG. 8 is an exploded view of the completed inkjet head 300 and FIG. 9 is a partially enlarged side view of the inkjet head 300. As seen from FIG. 8, the inkjet head 300 of the present invention comprises a pressure chamber plate 310, a piezo-electric element 320, a nozzle plate 330, a resin film 340 and a protective layer 350. The nozzle plate 330 corresponds to the nozzle plate 10 shown in FIG. 1 and the pressure chamber plate 310 corresponds to the pressure chamber plate 30 shown in FIG. 1. The pressure chamber plate 310, the resin film 340 and the protective layer 350 are aligned with each other at a nozzle connection surface 360 that is a surface to which a surface 330a of the nozzle plate 330 is connected. In other words, the front surface 310a of the pressure chamber plate 310, a front surface 340a of the resin film 340 and a front surface 350a of the protective layer 350 form the flat nozzle connection surface 360.

30 The pressure-chamber plate 310 has the desired number (four in FIG. 8 for description purposes) of pressure chambers 312 and ink introduction channels 314 and a common ink chamber 316 in an approximately rectangular parallelepiped glass plate. Each pressure chamber 312 receives and accommodates ink, and jets the ink from a nozzle 332 connected to an opening 312a as its internal pressure increases. The internal pressure changes according as the piezo-electric block 321 just under the pressure chamber 312 deforms, as will be described later. The pressure chamber 312 is formed as an approximately rectangular parallelepiped space by a concave groove on the pressure chamber plate 310 and the elastically deformable resin film 340. The common ink chamber 316 supplies ink to each pressure chamber 312 via the corresponding ink introduction channel 314. A bottom of the common ink chamber 316 is defined by the resin film 340 so as to absorb sudden internal pressure changes, and connected to an ink feed device (not shown) at a side surface 310b of the pressure chamber plate 310. The common ink chamber 316 supplies a necessary amount of ink to the pressure chamber 312 via the ink introduction channel 314 when the pressure chamber 312 returns to the original state after the chamber 312 contracts, receives pressure and jets ink.

40 50 60 70 80 90 100 110 120 130 140 150 160 170 180 190 200 210 220 230 240 250 260 270 280 290 300 310 320 330 340 350 360 370 380 390 400 410 420 430 440 450 460 470 480 490 500 510 520 530 540 550 560 570 580 590 600 610 620 630 640 650 660 670 680 690 700 710 720 730 740 750 760 770 780 790 800 810 820 830 840 850 860 870 880 890 900 910 920 930 940 950 960 970 980 990 1000 1010 1020 1030 1040 1050 1060 1070 1080 1090 1100 1110 1120 1130 1140 1150 1160 1170 1180 1190 1200 1210 1220 1230 1240 1250 1260 1270 1280 1290 1300 1310 1320 1330 1340 1350 1360 1370 1380 1390 1400 1410 1420 1430 1440 1450 1460 1470 1480 1490 1500 1510 1520 1530 1540 1550 1560 1570 1580 1590 1600 1610 1620 1630 1640 1650 1660 1670 1680 1690 1700 1710 1720 1730 1740 1750 1760 1770 1780 1790 1800 1810 1820 1830 1840 1850 1860 1870 1880 1890 1900 1910 1920 1930 1940 1950 1960 1970 1980 1990 2000 2010 2020 2030 2040 2050 2060 2070 2080 2090 2100 2110 2120 2130 2140 2150 2160 2170 2180 2190 2200 2210 2220 2230 2240 2250 2260 2270 2280 2290 2300 2310 2320 2330 2340 2350 2360 2370 2380 2390 2400 2410 2420 2430 2440 2450 2460 2470 2480 2490 2500 2510 2520 2530 2540 2550 2560 2570 2580 2590 2600 2610 2620 2630 2640 2650 2660 2670 2680 2690 2700 2710 2720 2730 2740 2750 2760 2770 2780 2790 2800 2810 2820 2830 2840 2850 2860 2870 2880 2890 2900 2910 2920 2930 2940 2950 2960 2970 2980 2990 3000 3010 3020 3030 3040 3050 3060 3070 3080 3090 3100 3110 3120 3130 3140 3150 3160 3170 3180 3190 3200 3210 3220 3230 3240 3250 3260 3270 3280 3290 3300 3310 3320 3330 3340 3350 3360 3370 3380 3390 3400 3410 3420 3430 3440 3450 3460 3470 3480 3490 3500 3510 3520 3530 3540 3550 3560 3570 3580 3590 3600 3610 3620 3630 3640 3650 3660 3670 3680 3690 3700 3710 3720 3730 3740 3750 3760 3770 3780 3790 3800 3810 3820 3830 3840 3850 3860 3870 3880 3890 3900 3910 3920 3930 3940 3950 3960 3970 3980 3990 4000 4010 4020 4030 4040 4050 4060 4070 4080 4090 4100 4110 4120 4130 4140 4150 4160 4170 4180 4190 4200 4210 4220 4230 4240 4250 4260 4270 4280 4290 4300 4310 4320 4330 4340 4350 4360 4370 4380 4390 4400 4410 4420 4430 4440 4450 4460 4470 4480 4490 4500 4510 4520 4530 4540 4550 4560 4570 4580 4590 4600 4610 4620 4630 4640 4650 4660 4670 4680 4690 4700 4710 4720 4730 4740 4750 4760 4770 4780 4790 4800 4810 4820 4830 4840 4850 4860 4870 4880 4890 4900 4910 4920 4930 4940 4950 4960 4970 4980 4990 5000 5010 5020 5030 5040 5050 5060 5070 5080 5090 5100 5110 5120 5130 5140 5150 5160 5170 5180 5190 5200 5210 5220 5230 5240 5250 5260 5270 5280 5290 5300 5310 5320 5330 5340 5350 5360 5370 5380 5390 5400 5410 5420 5430 5440 5450 5460 5470 5480 5490 5500 5510 5520 5530 5540 5550 5560 5570 5580 5590 5500 5510 5520 5530 5540 5550 5560 5570 5580 5590 5600 5610 5620 5630 5640 5650 5660 5670 5680 5690 5700 5710 5720 5730 5740 5750 5760 5770 5780 5790 5800 5810 5820 5830 5840 5850 5860 5870 5880 5890 5800 5810 5820 5830 5840 5850 5860 5870 5880 5890 5900 5910 5920 5930 5940 5950 5960 5970 5980 5990 5900 5910 5920 5930 5940 5950 5960 5970 5980 5990 6000 6010 6020 6030 6040 6050 6060 6070 6080 6090 6100 6110 6120 6130 6140 6150 6160 6170 6180 6190 6200 6210 6220 6230 6240 6250 6260 6270 6280 6290 6300 6310 6320 6330 6340 6350 6360 6370 6380 6390 6400 6410 6420 6430 6440 6450 6460 6470 6480 6490 6500 6510 6520 6530 6540 6550 6560 6570 6580 6590 6600 6610 6620 6630 6640 6650 6660 6670 6680 6690 6700 6710 6720 6730 6740 6750 6760 6770 6780 6790 6800 6810 6820 6830 6840 6850 6860 6870 6880 6890 6900 6910 6920 6930 6940 6950 6960 6970 6980 6990 7000 7010 7020 7030 7040 7050 7060 7070 7080 7090 7100 7110 7120 7130 7140 7150 7160 7170 7180 7190 7200 7210 7220 7230 7240 7250 7260 7270 7280 7290 7300 7310 7320 7330 7340 7350 7360 7370 7380 7390 7400 7410 7420 7430 7440 7450 7460 7470 7480 7490 7500 7510 7520 7530 7540 7550 7560 7570 7580 7590 7600 7610 7620 7630 7640 7650 7660 7670 7680 7690 7700 7710 7720 7730 7740 7750 7760 7770 7780 7790 7800 7810 7820 7830 7840 7850 7860 7870 7880 7890 7900 7910 7920 7930 7940 7950 7960 7970 7980 7990 8000 8010 8020 8030 8040 8050 8060 8070 8080 8090 8100 8110 8120 8130 8140 8150 8160 8170 8180 8190 8200 8210 8220 8230 8240 8250 8260 8270 8280 8290 8300 8310 8320 8330 8340 8350 8360 8370 8380 8390 8400 8410 8420 8430 8440 8450 8460 8470 8480 8490 8500 8510 8520 8530 8540 8550 8560 8570 8580 8590 8600 8610 8620 8630 8640 8650 8660 8670 8680 8690 8700 8710 8720 8730 8740 8750 8760 8770 8780 8790 8800 8810 8820 8830 8840 8850 8860 8870 8880 8890 8900 8910 8920 8930 8940 8950 8960 8970 8980 8990 9000 9010 9020 9030 9040 9050 9060 9070 9080 9090 9100 9110 9120 9130 9140 9150 9160 9170 9180 9190 9200 9210 9220 9230 9240 9250 9260 9270 9280 9290 9300 9310 9320 9330 9340 9350 9360 9370 9380 9390 9400 9410 9420 9430 9440 9450 9460 9470 9480 9490 9500 9510 9520 9530 9540 9550 9560 9570 9580 9590 9600 9610 9620 9630 9640 9650 9660 9670 9680 9690 9700 9710 9720 9730 9740 9750 9760 9770 9780 9790 9800 9810 9820 9830 9840 9850 9860 9870 9880 9890 9800 9810 9820 9830 9840 9850 9860 9870 9880 9890 9900 9910 9920 9930 9940 9950 9960 9970 9980 9990 10000 10010 10020 10030 10040 10050 10060 10070 10080 10090 10010 10020 10030 10040 10050 10060 10070 10080 10090 10100 10110 10120 10130 10140 10150 10160 10170 10180 10190 10110 10120 10130 10140 10150 10160 10170 10180 10190 10200 10210 10220 10230 10240 10250 10260 10270 10280 10290 10210 10220 10230 10240 10250 10260 10270 10280 10290 10300 10310 10320 10330 10340 10350 10360 10370 10380 10390 10310 10320 10330 10340 10350 10360 10370 10380 10390 10400 10410 10420 10430 10440 10450 10460 10470 10480 10490 10410 10420 10430 10440 10450 10460 10470 10480 10490 10500 10510 10520 10530 10540 10550 10560 10570 10580 10590 10510 10520 10530 10540 10550 10560 10570 10580 10590 10600 10610 10620 10630 10640 10650 10660 10670 10680 10690 10610 10620 10630 10640 10650 10660 10670 10680 10690 10700 10710 10720 10730 10740 10750 10760 10770 10780 10790 10710 10720 10730 10740 10750 10760 10770 10780 10790 10800 10810 10820 10830 10840 10850 10860 10870 10880 10890 10810 10820 10830 10840 10850 10860 10870 10880 10890 10900 10910 10920 10930 10940 10950 10960 10970 10980 10990 10910 10920 10930 10940 10950 10960 10970 10980 10990 11000 11010 11020 11030 11040 11050 11060 11070 11080 11090 11010 11020 11030 11040 11050 11060 11070 11080 11090 11100 11110 11120 11130 11140 11150 11160 11170 11180 11190 11110 11120 11130 11140 11150 11160 11170 11180 11190 11200 11210 11220 11230 11240 11250 11260 11270 11280 11290 11210 11220 11230 11240 11250 11260 11270 11280 11290 11300 11310 11320 11330 11340 11350 11360 11370 11380 11390 11310 11320 11330 11340 11350 11360 11370 11380 11390 11400 11410 11420 11430 11440 11450 11460 11470 11480 11490 11410 11420 11430 11440 11450 11460 11470 11480 11490 11500 11510 11520 11530 11540 11550 11560 11570 11580 11590 11510 11520 11530 11540 11550 11560 11570 11580 11590 11600 11610 11620 11630 11640 11650 11660 11670 11680 11690 11610 11620 11630 11640 11650 11660 11670 11680 11690 11700 11710 11720 11730 11740 11750 11760 11770 11780 11790 11710 11720 11730 11740 11750 11760 11770 11780 11790 11800 11810 11820 11830 11840 11850 11860 11870 11880 11890 11810 11820 11830 11840 11850 11860 11870 11880 11890 11900 11910 11920 11930 11940 11950 11960 11970 11980 11990 11910 11920 11930 11940 11950 11960 11970 11980 11990 12000 12010 12020 12030 12040 12050 12060 12070 12080 12090 12010 12020 12030 12040 12050 12060 12070 12080 12090 12100 12110 12120 12130 12140 12150 12160 12170 12180 12190 12110 12120 12130 12140 12150 12160 12170 12180 12190 12200 12210 12220 12230 12240 12250 12260 12270 12280 12290 12210 12220 12230 12240 12250 12260 12270 12280 12290 12300 12310 12320 12330 12340 12350 12360 12370 12380 12390 12310 12320 12330 12340 12350 12360 12370 12380 12390 12400 12410 12420 12430 12440 12450 12460 12470 12480 12490 12410 12420 12430 12440 12450 12460 12470 12480 12490 12500 12510 12520 12530 12540 12550 12560 12570 12580 12590 12510 12520 12530 12540 12550 12560 12570 12580 12590 12600 12610 12620 12630 12640 12650 12660 12670 12680 12690 12610 12620 12630 12640 12650 12660 12670 12680 12690 12700 12710 12720 12730 12740 12750 12760 12770 12780 12790 1271

transmit a deformation of each piezo-electric block 321 which will be described later to the corresponding pressure chamber 312 and to prevent ink in the pressure chamber 312 from penetrating into grooves 323 in the piezo-electric element 320. The resin film 340 is, for example, approximately 16  $\mu\text{m}$  thick and the order of Gpa adhesive. The resin film 340, which is a member that forms one surface of the pressure chamber 312, may be replaced with an elastic metal thin film.

The piezo-electric element 320 has layered structure having a plurality of (four in FIG. 1 for description purposes) piezo-electric blocks 321 which are divided by parallel grooves 323 which extend from a front surface 320a to a rear surface 320b. Internal electrodes 322 and 324 are provided between layers of piezoelectric blocks 321, and the internal electrode 322 is connected to an external electrode 326 and the internal electrode 324 is connected to an external electrode 328. FIG. 8 shows only one external electrode 328 for illustration purposes. As shown in FIG. 9, an active area 325 is a portion where the internal electrodes 322 and 324 overlap each other in direction A, and each piezo-electric block 321 deforms in the active area 325. The length of each active area 325 is adjustable depending upon a pressure to be applied to the pressure chamber 312. Since the active area 325 is spaced at a predetermined distance from the nozzle connection surface 360, even when the piezo-electric blocks 321 deform, such deformation does not affect the adhesion between the piezo-electric element 320 and the protective layer 350 at the nozzle connection surface 360.

The external electrode 326 is an electrode layer that is evaporated onto an entire surface of the front surface 320a of the piezo-electric element 320, and an external electrode commonly used for all the piezo-electric blocks 321. The external electrode 326 is grounded. On the contrary, the external electrode 328, which is provided on the rear surface 320b of the piezo-electric element 320, is however an electrode layer which is not evaporated onto an entire surface of the rear surface 320b and is independently provided only on a portion corresponding to each piezo-electric block 321. The external electrode 328 has no potential unless electrified, but may apply a positive voltage to the internal electrode 324.

Due to such a structure, each piezo-electric block 321 of the piezo-electric element 320 does not deform when no voltage is applied to the external electrode 328, since both potentials of the internal electrodes 322 and 324 remain zero. On the other hand, when a voltage is applied from the external electrode 328, each piezo-electric block 321 may deform in the direction A (longitudinal direction) in FIG. 8, independent of the other piezo-electric blocks 321. In other words, the direction A is the polarization direction of the piezo-electric blocks 321. When the electrification to the external electrode 328 stops, that is, when the piezo-electric element 320 is discharged, the corresponding piezo-electric block 321 returns to the original state.

The piezo-electric element 320 of this embodiment is made of a plurality of green sheets 327. Each green sheet 327 is blended with solvents such as a ceramic powder, etc., kneaded into a paste and then formed to be a thin film having a thickness of about 50  $\mu\text{m}$  by a doctor blade.

Among these green sheets, a pattern of the internal electrode 322 is printed and formed onto one surface of each of three green sheets, a pattern of the internal electrode 324 is printed and formed onto one surface of each of another three green sheets, and no internal electrode is formed onto

the remaining sheets. Each of the internal electrodes 322 and 324 is printed by blending alloy powder of silver and palladium with a solvent into a paste to apply for its pattern formation.

Then, the three sheets including the internal electrode 322 and the three sheets including the internal electrode 324 are alternately stuck together, and thereafter the remaining six sheets are also stuck together. Thereby, the layered structure of the piezo-electric element 320 is formed as shown in FIG. 9. The green sheets that include none of the internal electrode 322 or 324 are stuck at a lower portion (in FIG. 9) of the piezo-electric element 320 and form a base part. These layered green sheets are sintered. Then, at least six sheets are partially cut by a diamond cutter from the front surface 320a to the rear surface 320b, whereby a plurality of the piezo-electric blocks 321 divided by the grooves 323 is formed. Lastly, the external electrodes 326 and 328 are formed by vacuum evaporation at the front surface 320a and the rear surface 320b. It is possible to form the grooves 323 before sintering. The completed piezo-electric element 320 is submitted to a characteristic test by applying a voltage to the external electrodes 326 and 328, and malfunctioning ones are eliminated.

The inkjet head 300 shown in FIG. 8 further comprises the protective layer 350. The protective layer has useful effects as will be explained later, but there is a choice whether the protective layer is provided.

The protective layer 350 is a thermosetting epoxy adhesive member having an approximately rectangular parallelepiped shape with a thickness of about 50  $\mu\text{m}$ , and connected via a surface 350b to the front surface 320a of the piezo-electric element 320 (external electrode 326). The materials for the protective layer 350, however, are not limited to this type. For example, an epoxy filler member, an acrylic resin, a polyethylene resin or the like are usable for the protective layer 350. The protective layer 350 in the actual inkjet head 300 does not have a rectangular parallelepiped shape in the strict sense of the term, and an interface between the protective layer 350 and the piezo-electric element 320 is not clear or simple as shown in FIGS. 8 and 9 by the external electrode 326 and the surface 350b. The protective layer 350 partially penetrates through the grooves 323 into the piezo-electric element 320 before heatedly solidifying. Accordingly, it is preferable that the protective layer 350 is made of insulators so as to prevent a short circuit of the internal electrodes 322 and 324. The protective layer 350 of this embodiment is applied to the piezo-electric element 320 (external electrode 326) all over the front surface 320a, but may, if necessary, be applied partially.

The protective layer 350 spaces the piezo-electric element 320 about 50  $\mu\text{m}$  apart from the nozzle connection surface 360. If ink leaked from the pressure chamber 12 and penetrated into the piezo-electric element 320, the ink would penetrate into the piezo-electric element 320 mainly along the nozzle connection surface 360. However, the protective layer 350 spaces from the nozzle connection surface 360 the piezo-electric element which has been conventionally located on the nozzle connection surface 360, and thereby prevents the ink from penetrating into the piezo-electric element 320 and short-circuiting the internal electrodes 322 and 324.

Moreover, the protective layer 350 shields the grooves 323. If ink leaked and penetrated into the piezo-electric element 320, the ink would penetrate mainly from an opening 312a of the pressure chamber 312, running along the nozzle connection surface 360, through the grooves 323

into the piezo-electric element 320. However, the protective layer 350 does shield the grooves 323 against or from the nozzle connection surface 360, and thereby prevents the ink from penetrating into the groove 323 from somewhere in the neighborhood of the front surface 320a of the piezo-electric element 320 and short-circuiting the internal electrodes 322 and 324.

In addition, the protective layer 350 also has the effect of protecting the piezo-electric element 320 from being destroyed by polishing in a polishing process for forming the nozzle connection surface 320a among various steps of manufacturing the inkjet head. Consequently, the polishing process never causes any removing crack and chip-off of the piezo-electric element 320. The external electrode is never cut off. Furthermore, the pressure chamber plate 310, which is made of glass, is rather strong, and thereby enables such a high polishing speed as to shorten the polishing time down to about one-fifth in comparison with conventional manufacturing methods.

The nozzle plate 330 is made of metal, e.g. stainless steel, etc. Each nozzle 332 may be formed, as described above with reference to FIG. 6, with a punch using a pin or the like, preferably into a conic shape (or as showing a tapering section) spreading from the front surface 330b toward the rear surface 330a of the nozzle plate 330. To obtain such a conic shaped nozzle 332 is one of the reasons why the pressure chamber plate 310 and the nozzle plate 330 are not formed in one but the nozzle plate 330 is adhered to the pressure chamber plate 310. In this embodiment, the nozzle 332 is about 80  $\mu\text{m}$  in diameter at the rear surface 330a and about 25 through 35  $\mu\text{m}$  at the front surface 330b. The present invention is also applicable to such an inkjet head that a nozzle thereof is formed, for example, above the pressure chamber plate 310 shown in FIG. 8, unlike the inkjet head 300.

On the surface (front surface) 330b of the nozzle plate 330, at least around the nozzle 332, is formed the water-repellent coating 100. Of course, the water-repellent coating 100 may be formed all over the front surface 330b. The water-repellent coating serves to stabilize a wiping operation, which will be described later, and to provide a high quality image. It is to be construed that the water-repellent coating should be located differently to accompany the nozzle where the nozzle of the inkjet head is formed, for example, above the pressure chamber plate 310 shown in FIG. 8.

In the inkjet head 300, each external electrode 328 independently applies a voltage to the internal electrode 324 of the piezo-electric block 321, and each piezo-electric block 321 independently deforms in the direction A in FIG. 1, bending the resin film 340 in the direction A and compressing the corresponding pressure chamber 312. This compression results in jetting ink from the pressure chamber 321 through the corresponding nozzle 332. When the electrification from the external electrode 328 stops, the resin film 340 and the piezo-electric block 321 returns to the original states by discharging. At that time, the internal pressure of the pressure chamber 312 reduces and ink is supplied from the common ink chamber 316 through the ink introduction channel 314 to the pressure chamber 312.

Although this embodiment uses the piezo-electric element 320 that deforms in the longitudinal direction, but another embodiment may use one that deforms in the lateral direction. Further, the present invention is not limited to the piezo-type inkjet head employing the piezo-electric element but applicable to the bubble-type inkjet head.

Referring next to FIG. 10, a description will be given of an inkjet printer 400 provided with the inkjet head 300 of the present invention. In each drawing, those members designated by the same reference numeral denote the same members, and a duplicate description will be omitted. FIG. 10 schematically illustrates an embodiment of the color inkjet printer (recording device) 400 to which the inkjet head 300 of the present invention is applied. In a housing 410 of the recording device 400, a platen 414 is rotatably provided.

In a recording operation, the platen 412 is driven to intermittently rotate by a driving motor 414 and send recording paper P at a predetermined feed pitch in the arrow direction W. In the housing 416 of the recording device, a guide rod 416 is provided in parallel to and above the platen 412.

A carriage 418 is mounted to an endless driving belt 420 that is driven by the driving motor 422 reciprocating for scanning along the platen 412.

The carriage 412 is mounted with a black recording head 424 and a color recording head 426. The color recording head 426 may comprise three parts. The black recording head 424 is removably provided with a black ink tank 428, and the color recording head 426 is removably provided with color ink tanks 430, 432 and 434. The inkjet head 300 of the present invention is applicable to such recording heads 424 and 426.

Needless to say, the black ink tank 428 accommodates black ink and the color ink tanks 430, 432 and 434 accommodate yellow ink, cyan ink and magenta ink respectively.

While the carriage 418 reciprocates along the platen 412, the black recording head 424 and the color recording head 426 are driven based on image data received from a word processor and a personal computer, etc., predetermined characters, images and the like are recorded on recording paper P. When the recording operation is suspended, the carriage 418 is returned to its home position and this home position is provided with a nozzle maintenance mechanism (or backup unit) 436.

The nozzle maintenance mechanism 436 is provided with a movable suction cap (not shown) and a suction pump (not shown) connected to the movable suction cap. When the recording heads 224 and 226 are placed at the home position, the suction cap is adsorbed to the nozzle plate of each recording head and the nozzle of the nozzle plate is sucked. This mechanism prevents the nozzle from being plugged. After that, a wiping unit (also not shown) wipes out the nozzle plate 330b with a wiper. On that occasion, the water-repellent coating 100 wipes out ink on the nozzle plate surface 330b completely, and the hard body 108 in the water-repellent coating 100 prevents the water-repellent coating from being destroyed or otherwise.

Although the preferred embodiments of the present invention have been described above, it is to be understood that various modifications and changes may be made in the present invention without departing from the spirit and scope thereof.

According to the water-repellent coating as set forth in claim 1, the water repellency of its fluorocarbon polymer works well serving to provide a high quality image, and its hard body enhancing the wiping resistance of the fluorocarbon polymer guarantees to continuously provide the high quality image. According to the water-repellent coating as set forth in claim 2, its flat hard body is not so vulnerable to friction or likely to fall off compared with a spherical hard body, and therefore can keep its wiping resistance for a long time. According to the water-repellent coating as set forth in claim 3, its flat

13

body having a big particle diameter never prevents the nozzle plate surface from being smoothly wiped. According to the water-repellent coating as set forth in claims 4 and 5, the flat hard body applicable to claim 1 is easily obtainable. The water-repellent coating as set forth in claims 6 and 7 can be easily formed without any special plating process. The recording device as set forth in claim 8 including the same water-repellent coating as claimed in claims 1 through 7 have the same effect as these claims.

The method of forming the water-repellent coating as set forth in claim 9 enables the hard body to protrude from the water-repellent coating surface; therefore, the wiping resistance of the water-repellent coating is advantageously enhanced. According to the method of forming the water-repellent coating as set forth in claim 10, the fluoric polymer melts by the heat treatment taking in the additive hard body whereby sufficient water repellency is expected even on the surface of the intrinsically low water-repellent hard body.

What is claimed is:

1. A print head comprising:  
a nozzle plate including a nozzle which jets ink; and  
a water-repellent coating which is formed on said nozzle plate as a substrate around said nozzle and comprises a fluoric polymer formed by a plating process and a hard body protecting said fluoric polymer.
2. A print head according to claim 1 wherein said hard body has a flat shape.
3. A print head according to claim 1 wherein a major axis of a particle diameter of said hard body does not exceed 1  $\mu\text{m}$ .
4. A print head according to claim 1 wherein said hard body includes a boron nitride single crystal.

14

5. A print head according to claim 1 wherein said hard body includes a boron carbide single crystal.

6. A print head according to claim 1 wherein an electrolytic plating process is adopted as said plating process.

7. A print head according to claim 1 wherein an electroless plating process is adopted as said plating process.

8. A recording device comprising:

a print head; and

a driving device which drives said print head wherein said print head includes:

a nozzle plate including a nozzle which jets ink; and  
a water-repellent coating which is formed on said nozzle plate as a substrate around said nozzle and comprises a fluoric polymer formed by a plating process and a hard body protecting said fluoric polymer.

9. A method of forming a water-repellent coating comprising the steps of:

forming a resist onto a nozzle plate while partially projecting the resist from the nozzle outwardly;  
performing a strike deposit via the resist;  
performing a water-repellent coating containing a plated coating, a fluoric polymer and a hard body protecting said fluoric polymer via the resist; and  
removing the resist.

10. A method of forming a water-repellent coating according to claim 9 further comprising the step of heating said water-repellent coating until a water repellency of said water-repellent coating becomes enough to make a contact angle of ink containing 10% of alcohol 60 degrees or larger.

\* \* \* \* \*